# EUROPEAN PATENT SPECIFICATION

(11) **EP 1 893 733 B1**
(45) Date of publication and mention of the grant of the patent: **02.06.2010**
(21) Application number: 06841253.5
(22) Date of filing: 14.06.2006
(51) Int. Cl.: C11D 3/37, C11D 11/00

(54) **COMPOSITIONS CONTAINING A POLYORGANOSILOXANE HAVING ONE OR MORE PIPERIDINYL FUNCTIONS AS A PROTECTANT FOR SURFACES**
ZUSAMMENSETZUNGEN MIT EINEM POLYORGANOSILOXAN MIT EINER ODER MEHRERER PIPERIDINYLFUNKTIONEN ALS OBERFLÄCHENSCHUTZMITTEL
COMPOSITIONS CONTENANT UN POLYORGANOSILOXANE COMPRENANT UNE OU PLUSIEURS FONCTIONS PIPERIDINYLE EN TANT QU AGENT DE PROTECTION DE SURFACES

(30) Priority: 24.06.2005 US 693696 P
(43) Date of publication of application: 05.03.2008
(73) Proprietor: BASF SE, 67056 Ludwigshafen (DE)
(72) Inventor: JAYNES, Bingham Scott, New City, NY 10956 (US); CHROBACZEK, Harald, 86153 Augsburg (DE)
(86) International application number: PCT/EP2006/063172
(87) International publication number: WO 2007/054381

(56) References cited:
- EP-A- 0 659 930
- WO-A-96/21696
- WO-A-97/33034
- FR-A- 2 824 841
- US-B1- 6 328 912

## Description

The present invention relates to the use of cleaning/protectant compositions containing a polyorganosiloxane having one or more piperidinyl functions in the protection of vinyl and other surfaces from environmental exposure such as UV- or oxidation-induced damage.

### BACKGROUND

This invention concerns the use of compositions containing a polyorganosiloxane having one or more piperidinyl groups in order to protect vinyl and other surfaces from environmental exposure such as UV-induced or oxidation-induced damage.

The use of silicon-based compositions has already been suggested for the treatment of laundry made of textile fibers. More specifically, the addition of amino-silicones to washing or rinsing compositions has been suggested, e.g. in U.S. Patent No. 4,585,563; WO 92/07927; WO 98/39401 and EP-A-150872, in order to produce a softening effect. Other perceptible effects, such as anti-static, anti-wrinkling and ease-of-ironing can also result. The described amino-functions, which are linked to a silicon atom by means of an alkylene bridge containing from 1 to 6 carbon atoms, are of the -N(X)(Y) type, where the symbols X and Y independently represent H, a C₁-C₃alkyl radical, a phenyl radical, a C₅-C₆cycloalkyl radical, a -C₁-C₆-alkylene-NH₂ radical, or a -COR radical, where R is a monovalent hydrocarbon radical. Amino-modified silicones, including those modified with piperidinyl functionality are also disclosed as fabric softening agents in U.S. Patent Nos. 6,800,602; 6,815,412; 6,825,683; 6,831,055; and in FR 2,824,841.

Polyvinyl chloride (PVC) protectants that have been commercialized over the years often comprise solutions or emulsions of polydimethylsiloxanes and various other additives such as those described in US patent Nos. 3,956,174 and 5,183,845. The products are commonly used for automotive interior and exterior PVC (vinyl) parts as well as household vinyl or other plastic products to improve the appearance by providing gloss, and to protect the surface by improving durability and water repellency. While these products provide temporary improvements to vinyl and plastic surfaces, testing has shown that single applications of these products do not effectively protect vinyl from extended weathering and exposure to UV light.

Efforts have been made to manufacture vinyl products that are resistant to the deleterious effects of UV light by incorporating additives such as hindered amine light stabilizers (HALS) directly into the vinyl resin during the manufacturing process. For example, the use of HALS in the manufacture of a variety of organic polymers is described in US patent Nos. 4,472,547; 4,547,537, and 5,241,067. However, these additives do not afford the long-term protection to the substrate that is needed for vinyl products that are constantly exposed to UV light such as upholstery for automobiles and boats, vinyl car tops, etc.

Efforts have also been made to incorporate HALS molecules directly into vinyl protectant formulations in order to provide an additional amount of protectant each time the surface is treated. Polysiloxane emulsion compositions containing HALS components are described in WO 96/21696. While these compositions provide suitable temporary protection, the HALS is easily removed from the surface by wiping or wear so that the protective effect is lost. The HALS molecules have also been found to migrate downward into the substrate away from the surface requiring protection, and thus diminishing the protective power of the remaining siloxane coating.

### SUMMARY OF THE INVENTION

Surprisingly it has now been found that a polyorganosiloxane having one or more piperidinyl groups bound to the polyorganosiloxane can provide durable protection against weathering and exposure to UV light to hard surfaces such as vinyl and plastic surfaces.

The present invention is a method of protection of a hard surface, which comprises contacting said hard surface with an effective amount of a protectant formulation containing a polyorganosiloxane having one or more piperidinyl groups bound to the polyorganosiloxane.

### DETAILED DESCRIPTION OF THE INVENTION

The present invention concerns the use of a protectant and surface cleaning composition for protecting hard surfaces, wherein the composition contains a polyorganosiloxane having one or more piperidinyl groups bound to the polyorganosiloxane. Said piperidinyl groups may be bonded directly or indirectly to the siloxane backbone or to a terminal group.

The treatment composition used in the present method comprises at least one polyorganosiloxane, which includes at least one group of the formula:

(R)ₐ(X)_{b}RₚSi(O) [3 - (a+b)]/2 (I)

wherein
- the R groups can be the same or different, and represent monovalent linear or branched C₁-C₄ alkyl, phenyl or 3,3,3-trifluoro propyl radicals;
- the X groups can be the same or different, and represent monovalent linear or branched hydroxyalkyl groups, hydroxyl groups, or C₁-C₃ alkoxy radicals;
- Rₚ represents one or more sterically hindered piperidinyl groups selected from
   ◆ the radicals of formula (II): in which
      - R⁴ is a divalent hydrocarbon radical selected from:
         - linear or branched alkylene radicals with between 2 and 18 carbon atoms;
         - alkylene-carbonyl radicals whose linear or branched alkylene stems have between 2 and 20 carbon atoms;
      - alkylene-cyclohexylene radicals whose linear or branched stems have between 2 and 12 carbon atoms, and whose cyclohexylene stem includes an OH group and, optionally, 1 or 2 alkyl radicals with between 1 to 4 carbon atoms;
      - radicals according to the formula -R⁷- O - R⁷- wherein the identical or varying R⁷ radicals represent alkylene radicals with 1 to 12 carbon atoms;
         • radicals according to the formula -R⁷ - O - R⁷- in which the R⁷ radicals have the aforementioned values, and one or both are substituted with one or two -OH groups;
         • radicals according to the formula -R⁷ - COO - R⁷- in which the R⁷ radicals have the aforementioned values;
         • radicals according to the formula - R⁸ - O - CO - R⁹- in which the identical or different R⁸ and R⁹ radicals represent alkylene radicals with between 2 and 12 carbon atoms, and where the radical R⁸ or R⁹ can optionally be substituted with a hydroxyl radical;
         • U represents -O- or -NR¹⁰-, R¹⁰ being a radical selected from a hydrogen atom, a linear or branched alkyl radical with between 1 and 6 carbon atoms, or a divalent radical, according to the following formula: in which R⁴ is as defined above, R⁵ and R⁶ have the following values, and R¹¹ represents a linear or branched divalent alkylene radical with between 1 and 12 carbon atoms, and where R¹¹ is connected to an -NR¹⁰- radical, and the R⁴ is connected to a silicon atom;
         - radicals R⁵, whose values can be identical or different, are linear or branched alkyl radicals having between 1 and 3 carbon atoms or phenyl radicals;
         • radical R⁶ represents either hydrogen, a radical R⁵ or O^{•};
   ◆ and the remaining formula radicals (III):
      - where R^{'4} is a trivalent radical having the following formula: where m is between 2 and 20, or a trivalent radical having the following formula: where p is between 2 and 20;
      - U' represents -O- or NR¹², where R¹² is hydrogen or a linear or branched alkyl radical with between 1 and 6 carbon atoms;
      - R⁵ and R⁶ have the same values as those indicated in Formula (II), wherein;
- a is 0, 1, or 2;
- b is 0, 1, or 2;
- and where "a + b" can not be more than 2.

Polyorganosiloxanes with sterically hindered amino functions as shown in Formula (I) can be obtained according to the process described in EP-A-659930.

These can have a dynamic viscosity ranging from approximately 100 mPa.s to 200,000 mPa.s at 25°C as measured for example with a Brookfield viscometer.

In one embodiment, said polyorganosiloxane with sterically hindered amino functions is a linear, cyclic or branched polyorganosiloxane according to formula (I'): wherein:
(1) the values of Z, identical or not, represent R¹, and/or Rₚ;
(2) the values of R¹, R² and R³, identical and/or not, represent a monovalent hydrocarbon radical selected from a range of linear or branched alkyl radicals with between 1 and 4 carbon atoms, linear or branched alkoxy radicals with between 1 and 4 carbon atoms, phenyl radicals, hydroxyl, methoxy and methyl radicals;
(3) the value of Rₚ, be it for identical or different functional groups, represents a group with one or more sterically hindered piperidinyl functions, selected from those in Formulas (II) or (III) above; and
(4) included are between 10 and 450 Si-containing units without Rₚ groups;
   - and from 1 to 10 Si-containing units with Rₚ -type groupings;
   - 0 ≤ w ≤10, and 8 < (x+y) < 448.

R¹, R² and R³ preferably represent hydroxyl, methoxy or methyl radicals.

The polysiloxane of formula (1') preferably includes between 5 and 250 Si-containing units without Rₚ groups and preferably 1 to 10 Si-containing units with Rₚ -type groupings.

An objective of this invention is to define a method for improving the properties of a composition designed for protecting hard surfaces, such as vinyl or other plastic surfaces, by adding to the composition at least one polyorganosiloxane with sterically hindered amino functions, according to Formulas (I) or (I'), in sufficient quantity to provide a UV protection effect.

Such compositions can be in various forms, but are generally emulsions of organopolysiloxanes, or silicone fluids, in water. The organopolysiloxanes are preferably dimethylsiloxane polymers, linear in nature. The dimethylpolysiloxane fluids suitable for use have a viscosity range of 10 to 100,000 centistokes. Preferably, the viscosity of the silicone fluid used should be in the range of from about 100 to 10,000 centistokes. By substitution of some of the methyl groups with other organic or organofunctional groups, other organopolysiloxanes can be produced, and are suitable for use in this composition. For example, amino-modified polysiloxanes may be used.

The silicone fluid or mixture of fluids is typically used in the form of a water emulsion, where water represents from about 30% to 99% of the total weight of formulation. Such silicone fluids and emulsions of these in water are described in detail in US patent Nos. 3,956,174 and 5,183,845, both incorporated herein by reference.

The silicone fluid of the protectant composition is comprised at least in part of piperidinyl (HALS) substituted polysiloxane polymers as described in this invention. The HALS substituted polymer can represent any portion from 0.1 % to 100% by weight of the total amount of polysiloxane present in the protectant formulation, so long as the amount of HALS-containing component is sufficient to provide protection to the surface being treated. The preferred amount of HALS-substituted polymer is 10-100% by weight with respect to total amount of polysiloxane, and the most preferred amount is 40-100% by weight.

Additional components of the protectant formulation may include a variety of materials familiar to those skilled in the art. These additives may include, but are not limited to: water, organic solvents, emulsifiers (to provide stability to the emulsion), other surfactants and wetting agents (to aid wetting and facilitate breaking of the emulsion upon application), glycerin, ethylene glycol, propylene glycol, other glycols, dyes, fragrances, foam inhibitors, UV absorbers, stabilizers, preservatives, rust inhibitors rust inhibitors, other adjuvant materials, and mixtures thereof.

The method of use of the protectant compositions of this invention comprises application of the composition onto a hard surface to be protected by spraying, wiping, or other similar means.

The composition may also be first applied to a nonwoven fabric, wiping tool, or other implement suitable for the delivery of the composition onto the surface. The material is then allowed to thoroughly wet and coat the surface for some period of time. Any excess material may be wiped off if necessary, and the surface may be buffed to a shine if desired.

Preferably the protectant composition comprises at least one polyorganosiloxane of the formula (1) or (1') of this invention.

The term "hard surface" includes both rigid and flexible materials. Especially preferred are materials that have surfaces that are susceptible to UV or oxidative damage and that may be treated with a siloxane emulsion without harm to the surface. These include plastics (e.g. vinyl/PVC, Plexiglas/PMMA, other acrylics, styrenics, polyolefins, nylon, polyurethane, etc.), rubber, silicones and untreated wood; latex or oil-based paints and coatings (e.g. stains, polyurethanes, varnishes, shellacs) on various hard surfaces, especially wood; melamines, composites, paper-based surfaces such as wallpaper, and natural and synthetic leathers.

The following examples describe certain embodiments of this invention, but the invention is not limited thereto. These examples are not meant to limit the scope of the invention. Rather, the scope of the invention is to be determined only by the appended claims and their equivalents. In these examples all parts given are by weight unless otherwise indicated.

### EXAMPLE 1

Protectant Composition: A HALS-modified polysiloxane (C.A.S. registration #171543-65-0) with a nitrogen content of 0.38% was added at a level of 15% by weight to water. The approximate structure of the siloxane is shown below:

An emulsifier with a hydrophilic/lipophilic balance (HLB) of 12 was added at a level of 6% and the mixture was emulsified with a high-speed mixer. An appropriate amount of acid was added while stirring until the mixture became clear. Such an emulsion is commercially available as ULTRATEX^{®} FMW from Ciba Specialty Chemicals.

### EXAMPLE 2

Method of Treatment of vinyl: A silicone microemulsion in water comprising 15% of the HALS-substituted polydimethylsiloxane polymer from Example 1 was applied to three 7 cm x 14 cm pieces of automotive dashboard vinyl by adding 1 ml of the protectant formulation to the surface and wiping the material onto the vinyl with a cotton terry cloth for 15 seconds. Three vinyl pieces were treated in the same manner using a commercial protectant formulation. The treated vinyl swatches as well as a set of three untreated vinyl swatches were then placed in an Atlas Ci4000 Xenon Weatherometer and exposed to UV light using an interior automotive accelerated weathering program as specified in SAE-J-1885.

The vinyl surface was evaluated for degradation by first washing it thoroughly with a detergent solution, rinsing with deionized water and then air-drying. The vinyl was then analyzed using a Thermo Electron Avatar 370 FTIR spectrometer equipped with a Smart Orbit ATR accessory fitted with a diamond crystal. An absorption spectrum was recorded for each cleaned and dried vinyl sample, and the ratio of peak heights for the absorbance at ∼1250 cm⁻¹ and 1098 cm⁻¹ was calculated. The decrease in this peak ratio corresponds to the degradation of the polyurethane surface coating on the vinyl swatch. Thus, lower values of this ratio indicate a higher degree of degradation.

Degradation values for the treated and control vinyl swatches are presented in the table below, for a UV exposure time of 48 hr total (-90 kJ exposure energy). Samples treated with the emulsion from Example 1 had reduced degradation levels versus the control or those treated with the commercial protectant.

| Vinyl Treatment | Peak ratio, T = 0 | Peak ratio, T = 48 hrs |
|---|---|---|
| None | 1.49 | 0.65 |
| Commercial Protectant | 1.53 | 0.65 |
| Emulsion of Example 1 | 1.47 | 0.72 |

### EXAMPLE 3

Method of Treatment of vinyl. Vinyl swatches were treated in the same manner as in Example 2, except that the swatches were retreated with protectant after 16 and 32 hours of exposure in the Weatherometer. After a total of 48 hours of exposure (90 kJ of energy), the samples were washed, rinsed and dried, and analyzed by the IR method described in Example 2.

The peak ratios in the table below indicate that material treated with the emulsion from Example 1 again exhibited the lowest degree of degradation of the three samples tested:

| Vinyl Treatment | Peak ratio, T = 0 | Peak ratio, T = 48 hrs |
|---|---|---|
| None | 1.49 | 0.72 |
| Commercial Protectant | 1.49 | 0.75 |
| Emulsion of Example 1 | 1.50 | 0.76 |

## Claims

1. A method of protecting a hard surface, which comprises contacting said hard surface with a protectant composition containing an effective amount of a polyorganosiloxane having one or more piperidinyl groups bound to the polyorganosiloxane.

2. A method according to claim 1, which comprises contacting said hard surface with an effective protectant amount of a polyorganosiloxane of the formula
(R)ₐ(X)_{b}RₚSi(O) [3 - (a+b)]/2 (I)
wherein
- the R groups can be the same or different, and represent monovalent linear or branched C₁-C₄ alkyl, phenyl or 3,3,3-trifluoro propyl radicals;
- the X groups can be the same or different, and represent monovalent linear or branched hydroxyalkyl groups, hydroxyl groups, or C₁-C₃ alkoxy radicals;
- Rₚ represents one or more sterically hindered piperidinyl groups selected from
◆ the radicals of formula (II): in which
• R⁴ is a divalent hydrocarbon radical selected from:
• linear or branched alkylene radicals with between 2 and 18 carbon atoms;
• alkylene-carbonyl radicals whose linear or branched alkylene stems have between 2 and 20 carbon atoms;
• alkylene-cyclohexylene radicals whose linear or branched stems have between 2 and 12 carbon atoms, and whose cyclohexylene stem includes an OH group and, optionally, 1 or 2 alkyl radicals with between 1 to 4 carbon atoms;
• radicals according to the formula -R⁷ - O - R⁷- wherein the identical or varying R⁷ radicals represent alkylene radicals with 1 to 12 carbon atoms;
• radicals according to the formula -R⁷ - O - R⁷- in which the R⁷ radicals have the aforementioned values, and one or both are substituted with one or two -OH groups;
• radicals according to the formula -R⁷- COO - R⁷- in which the R⁷ radicals have the aforementioned values;
• radicals according to the formula - R⁸- O - CO - R⁹- in which the identical or different R⁸ and R⁹ radicals represent alkylene radicals with between 2 and 12 carbon atoms, and where the radical R⁸ or R⁹ can optionally be substituted with a hydroxyl radical;
• U represents -O- or -NR¹⁰-, R¹⁰ being a radical selected from a hydrogen atom, a linear or branched alkyl radical with between 1 and 6 carbon atoms, or a divalent radical, according to the following formula: in which R⁴ is as defined above, R⁵ and R⁶ have the following values, and R¹¹ represents a linear or branched divalent alkylene radical with between 1 and 12 carbon atoms, and where R¹¹ is connected to an -NR¹⁰- radical, and the R⁴ is connected to a silicon atom;
• radicals R⁵, whose values can be identical or different, are linear or branched alkyl radicals having between 1 and 3 carbon atoms or phenyl radicals;
• radical R⁶ represents either hydrogen, a radical R⁵ or O^{•};
◆ and the remaining formula radicals (III):
• where R^{'4} is a trivalent radical having the following formula: where m is between 2 and 20, or a trivalent radical having the following formula: where p is between 2 and 20;
• U' represents -O- or NR¹², where R¹² is hydrogen or a linear or branched alkyl radical with between 1 and 6 carbon atoms;
• R⁵ and R⁶ have the same values as those indicated in Formula (II), wherein;
- a is 0, 1, or 2;
- b is 0, 1, or 2;
- and where "a + b" cannot be more than 2.

3. A method according to claim 1, which comprises contacting said hard surface with an effective protectant amount of a polyorganosiloxane of the formula (I'): wherein:
(1) the values of Z, identical or not, represent R¹, and/or Rₚ;
(2) the values of R¹, R² and R³, identical and/or not, represent a monovalent hydrocarbon radical selected from a range of linear or branched alkyl radicals with between 1 and 4 carbon atoms, linear or branched alkoxy radicals with between 1 and 4 carbon atoms, phenyl radicals, hydroxyl, methoxyl and methyl radicals;
(3) the value of Rₚ, be it for identical or different functional groups, represents a group with one or more sterically hindered piperidinyl functions, selected from those in Formulas (II) or (III) above; and
(4) included are between 10 and 450 Si-containing units without Rₚ groups; and from 1 to 10 Si-containing units with Rₚ -type groupings; 0 ≤ w ≤10, and 8 < (x+y) < 448.

4. A method of protecting a hard surface according to any one of claim 1 to 3, wherein said surface is susceptible to UV or oxidative damage and may be treated with a siloxane emulsion without harm to the surface.

5. A method of protecting a hard surface according to any one of claims 1 to 4, wherein said surface is selected from plastics, rubber, silicones and untreated wood; painted and coated hard surfaces including wood; melamines and composites, paper-based surfaces, and natural and synthetic leathers.

## Patentansprüche

1. Verfahren zum Schützen einer harten Oberfläche, umfassend das Kontaktieren der harten Oberfläche mit einer schützenden Zusammensetzung, die eine wirksame Menge eines Polyorganosiloxans mit einer oder mehreren an das Polyorganosiloxan gebundenen Piperidinylgruppen enthält.

2. Verfahren gemäß Anspruch 1, umfassend das Kontaktieren der harten Oberfläche mit einer wirksamen schützenden Menge eines Polyorganosiloxans der Formel:
(R)ₐ(X)_{b}RₚSi(O) [3 - (a+b)]/2 (I)
worin
- die R-Gruppen gleich oder verschieden sein können und einwertige lineare oder verzweigte C₁-C₄-Alkyl-, Phenyl- oder 3,3,3-Trifluorpropylreste repräsentieren;
- die X-Gruppen gleich oder verschieden sein können und einwertige lineare oder verzweigte Hydroxyalkylgruppen, Hydroxylgruppen oder C₁-C₃-Alkoxyreste repräsentieren;
- Rₚ eine order mehrere sterisch gehinderte Piperidinylgruppen repräsentiert, gewählt aus
◆ den Resten der Formel (II) : worin
• R⁴ ein zweiwertiger Kohlenwasserstoffrest ist, gewählt aus:
• linearem oder verzweigten Alkylenresten mit zwischen 2 und 18 Kohlenstoffatomen;
• Alkylen-Carbonyl-Resten, deren lineare oder verzweigte Alkylenstämme bzw. -gerüste zwischen 2 und 20 Kohlenstoffatome aufweisen;
• Alkylen-Cyclohexylen-Resten, deren lineare oder verzweigte Gerüste zwischen 2 und 12 Kohlenstoffatome aufweisen und deren Cyclohexylengerüst eine OH-Gruppe und gegebenenfalls 1 oder 2 Alkylreste mit zwischen 1 bis 4 Kohlenstoffatomen einschließt;
• Reste gemäß der Formel -R⁷-O-R⁷, worin die identischen oder variierenden R⁷-Reste Alkylenreste mit 1 bis 12 Kohlenstoffatomen repräsentieren;
• Reste gemäß, der Formel -R⁷-O-R⁷, worin die R⁷-Reste die vorgenannten Werte haben und einer oder beide durch eine oder zwei -OH-Gruppen substituiert sind;
• Reste gemäß der Formel -R⁷-COO-R⁷, worin die R⁷-Reste die vorgenannten Werte haben;
• Reste gemäß, der Formel -R⁸-O-CO-R⁹, worin die identischen oder unterschiedlichen R⁸- und R⁹-Reste Alkylenreste mit zwischen 2 und 12 Kohlenstoffatomen repräsentieren und wobei der Rest R⁸ oder R⁹ gegebenenfalls mit einem Hydroxylrest substituiert sein kann;
• U für -O- oder -NR¹⁰- steht, wobei R¹⁰ ein Rest ist, welcher aus einem Wasserstoffatom, einem linearen oder verzweigten Alkylrest mit zwischen 1 und 6 Kohlenstoffatomen gewählt ist, oder ein zweiwertiger Rest ist, gemäß der nachstehenden Formel: worin R⁴ wie oben definiert ist, R⁵ und R⁶ die folgenden Werte haben und R¹¹ einen linearen oder verzweigten zweiwertigen Alkylenrest mit zwischen 1 und 12 Kohlenstoffatomen repräsentiert und worin R¹¹ mit einem -NR¹⁰-Rest verbunden ist und R⁴ mit einem Siliciumatom verbunden ist;
• Reste R⁵, deren Werte identisch oder verschieden sein können, lineare oder verzweigte Alkylreste mit zwischen 1 und 3 Kohlenstoffatomen oder Phenylreste sind;
• der Rest R⁶ entweder für Wasserstoff, einen Rest R⁵ oder O^{•} steht;
◆ und den restlichen Formelresten (III):
• worin R^{'4} ein dreiwertiger Rest mit der folgende Formel ist: worin m zwischen 2 und 20 ist, oder ein dreiwertiger Rest mit der folgenden Formol: worin p zwischen 2 und 20 ist;
• U' für -O- oder -NR¹² steht, worin R¹² Wasserstoff oder ein linearer oder verzweigter Alkylrest mit zwischen 1 und 6 Kohlenstoffatomen ist;
• R⁵ und R⁶ die gleichen Werte wie die in Formel (II) angegebenen haben, worin:
- a 0, 1 oder 2 ist;
- b 0, 1 oder 2 ist;
- und worin "a + b" nicht mehr als 2 sein können.

3. Verfahren gemäß Anspruch 1, umfassend das Kontaktieren der harten Oberfläche mit einer wirksamen schützenden Menge eines Polyorganosiloxans der Formel (I'): worin :
(1) die Werte von Z, die identisch sind oder nicht, R¹ und/oder Rₚ repräsentieren;
(2) die Werte von R¹, R² und R³, die identisch sind und/oder nicht, einen einwertigen Kohlenwasserstoffrest repräsentieren, welcher aus einem Bereich von linearen oder verzweigten Alkylresten mit zwischen 1 und 4 Kohlenstoffatomen, linearen oder verzweigten Alkoxyresten mit zwischen 1 und 4 Kohlenstoffatomen, Phenylresten, Hydroxyl-, Methoxyl- und Methylresten gewählt ist;
(3) der Wert von Rₚ, sei es für identische oder unterschiedliche funktionelle Gruppen, eine Gruppe mit einer oder mehreren sterisch gehinderten Piperidinylfunktionen repräsentiert, gewählt aus jenen in den Formeln (II) oder (III) weiter oben; und
(4) zwischen 10 und 450 Si-haltige Einheiten ohne Rₚ-Gruppen;
- und 1 bis 10 Si-haltige Einheiten mit Gruppierungen vom Rₚ-Typ eingeschlossen sind; 0 ≤ w ≤ 10 und 8 <(x+y)< 448.

4. Verfahren zum Schützen einer harten Oberfläche gemäß einem beliebigen der Ansprüche 1 bis 3, wobei die oberfläche für UV- oder oxidative Schädigung anfällig ist und mit einer Siloxan-Emulsion ohne Beschädigung der oberfläche behandelt werden kann.

5. Verfahren zum Schützen einer harten oberfläche gemäß einem beliebigen der Ansprüche 1 bis 4, wobei die Oberfläche aus Kunststoffen, Kautschuk, Silikonen und unbehandeltem Holz; lackierten und beschichteten harten Oberflächen einschließlich Holz; Melaminen und Verbundstoffen, Oberflächen auf Papierbasis und natürlichen und synthetischen Ledern gewählt ist.

## Revendications

1. Procédé de protection d'une surface dure, qui comprend la mise de ladite surface dure en contact avec une composition protectrice contenant une quantité efficace d'un polyorganosiloxane portant un ou plusieurs groupes pipéridinyle liés au polyorganosiloxane.

2. Procédé selon la revendication 1, qui comprend la mise de ladite surface dure en contact avec une quantité protectrice efficace d'un polyorganosiloxane de formule
(R)ₐ(X)_{b}RₚSi(O) [3-(a+b)]/2 (I)
dans laquelle
- les groupes R peuvent être identiques ou différents, et représentent des radicaux alkyle en C₁-C₄ monovalents linéaires ou ramifiés, phényle ou 3,3,3-trifluoropropyle ;
- les groupes X peuvent être identiques ou différents, et représentent des radicaux hydroxyalkyle monovalents linéaires ou ramifiés, hydroxyle ou alcoxy en C₁-C₃ ;
- Rₚ représente un ou plusieurs groupes pipéridinyle stériquement encombrés choisis parmi
■ les radicaux de formule (II) : dans laquelle
• R⁴ est un radical hydrocarboné divalent choisi parmi :
• les radicaux alkylène linéaires ou ramifiés portant entre 2 et 18 atomes de carbone ;
• les radicaux alkylène-carbonyle dont les branches alkylène linéaires ou ramifiées portent entre 2 et 20 atomes de carbones ;
• les radicaux alkylène-cyclohexylène dont les branches linéaires ou ramifiées postent entre 2 et 12 atomes de carbone, et dont la branche cyclohexylène comprend un groupe OH et, éventuellement, 1 ou 2 radicaux allyle portant entre 1 et 4 atomes de carbone ;
• les radicaux répondant à la formule -R⁷-O-R⁷-dans laquelle les radicaux R⁷, identiques ou différents, représentent des radicaux alkylène portant 1 à 12 atomes de carbone ;
• les radicaux répondant à la formule -R⁷-O-R⁷-dans laquelle les radicaux R⁷ prennent les valeurs susmentionnées, et l'un d'entre eux ou les deux sont substitués par un ou deux groupes -OH ;
• les radicaux répondant à la formule -R⁷-COO-R⁷-dans laquelle les radicaux R⁷ prennent les valeurs susmentionnées ; et
• les radicaux répondant à la formule -R⁸-O-CO-R⁹-dans laquelle les radicaux R⁸ et R⁹, identiques ou différents, représentent des radicaux alkylène portant entre 2 et 12 atomes de carbone, et le radical R⁸ ou R⁹ peut éventuellement être substitué par un radical hydroxyle ;
• U représente -O- ou -NR¹⁰-, R¹⁰ étant un radical choisi parmi un atome d'hydrogène, un radical alkyle linéaire ou ramifié portant entre 1 et 6 atomes de carbone, et un radical divalent répondant à la formule suivante : dans laquelle R⁴ est tel que défini ci-dessus, R⁵ et R⁶ prennent les valeurs ci-après, et R¹¹ représente un radical alkylène divalent linéaire ou ramifié portant entre 1 et 12 atomes de carbone, R¹¹ étant attaché à un radical -NR¹⁰-, et R⁴ étant attaché à un atome de silicium ;
• les radicaux R⁵, dont les valeurs peuvent être identiques ou différentes, sont des radicaux alkyle linéaires ou ramifiés portant entre 1 et 3 atomes de carbone ou des radicaux phényle ; et
• le radical R⁶ représente un hydrogène, un radical R⁵ ou O^{*} ;
• et les radicaux de formule (III) : dans laquelle
• R⁴ le est un radical trivalent répondant à la formule : où m est compris entre 2 et 20, ou un radical trivalent répondant à la formule : où p est compris entre 2 set 20 ;
• U' représente -O- ou NR¹², R¹² étant un hydrogène ou un radical alkyle linéaire ou ramifié portant entre 1 et 6 atomes de carbone ; et
• R⁵ et R⁶ prennent les mêmes valeurs que celles indiquées dans la formule (II) ;
- a vaut 0, 1 ou 2 ;
- b veut 0, 1 ou 2 ; et
- "a+b" ne peut pas être supérieur à 2.

3. Procédé selon la revendication 1, qui comprend la mise de ladite surface dure en contact avec une quantité protectrice efficace d'un polyorganosiloxane de formule (I') : dans laquelle
(1) les valeurs de Z, identiques ou différentes, représentent R¹ et/ou Rₚ ;
(2) les valeurs de R¹, R² et R³, identiques et/ou différentes, représentent un radical hydrocarboné monovalent choisi dans un groupe constitué par les radicaux allyle linéaires ou ramifiés portant entre 1 et 4 atomes de carbone, alcoxy linéaires ou ramifiés portent entre 1 et 4 atomes de carbone, phényle, hydroxyle, méthoxy et méthyle ;
(3) la valeur de Rₚ, que ce soit pour des groupes fonctionnels identiques ou différents, représente un groupe portant une ou plusieurs fonctions pipéridinyle stériquement encombrées, choisies parmi des formules (II) et (III) ci-dessus ; et
(4) sont inclus entre 10 et 450 motifs contenant du Si sans groupes Rₚ ; et
de 1 à 10 motifs contenant du Si avec des groupements de type Rₚ ;
0 ≤ w ≤ lu, et 8 < (x+y) < 448.

4. Procédé de protection d'une surface dure salon l'une quelconque des revendication 1 à 3, dans lequel ladite surface peut être endommagée par les trayons UV ou l'oxydation, et peut être traitée avec une émulsion de siloxane sans être endommagée.

5. Procédé de protection d'une surface dure selon l'une quelconque des revendications 1 à 4, dans lequel ladite surface est choisie parmi les plastiques, le caoutchouc, les silicones et le bols non traité ; les surfaces dures peintes et enduites, y compris le bois ; les mélaminés et les composites, les surfaces à base de 5 papier, et les cuirs naturels et synthétiques.
